

## UNITED STATES PATENT OFFICE

2,353,661

## PROCESS OF OBTAINING PHOTOGRAPHIC IMAGES

Béla Gáspár, Hollywood, Calif., assignor to  
Chromogen, Incorporated, a corporation of  
Nevada

No Drawing. Application December 7, 1940,  
Serial No. 369,123

5 Claims. (Cl. 95—88)

My invention relates to the production of photographic images and, more particularly, to the production of photographic reversal images.

It is common practice to produce photographic reversal images from a suitable emulsion of light-sensitive silver bromide by exposing a portion of it to produce a latent image therein, developing this image, and then, without fixing the image, removing the developed metallic silver deposit by an oxidizing agent without removing the unexposed silver bromide. The remaining silver bromide is then blackened by exposing it and developing it, or it may be converted by a chemical agent, such for example as sodium hydrosulphite.

In the known processes for the production of reversal images, the silver image first produced is removed either by a solution of sulphuric acid and potassium bichromate or a solution of sulphuric acid and potassium permanganate. Both of these solutions strongly affect the gelatin, or in the case of a paper support, the paper fiber; furthermore, they affect other substances such as sensitive and easily destroyable substances for coloring that may be contained in the emulsion. More particularly, they may affect dyes serving as filter dyes, sensitizing dyes or dyes serving later on in the process for the production of dye images. Likewise, in the case where a dye forming substance is used in the emulsion, they may affect the dye forming substance.

It is, therefore, an object of my invention to provide an improved method of treatment of the initial silver image contained in a photographic layer in a reversal process whereby the same may be bleached and removed without the use of strong acidic reactions or energetic oxidizing agents.

Another object of my invention is to provide an improved method of forming reversal images in photographic layers containing a developed silver image in a light-sensitive emulsion and a uniformly distributed substance for coloring which is sensitive to and is destroyed by known bleaching baths having acidic properties.

Another object of my invention is to provide such a method wherein the initial silver image in a reversal process is transformed into a silver salt and afterwards dissolved in a bath by the formation of a complex.

Another object of my invention is to provide such a method of forming reversal images wherein the initial silver image of a layer is treated to form a silver salt and the silver salt is later dissolved by the formation of a complex without de-

stroying or deleteriously affecting the coloring substance employed in the layer.

A further object of my invention is the provision of such a method in which the dissolution of the silver salt under complex formation does not result in the dissolution of the remaining silver bromide.

These and other objects of my invention will appear as the description proceeds, and its scope

will be pointed out in the claims appended hereto.

My invention will be best understood by an illustration of its application to an emulsion suitably adapted for the production of photographic reversal images.

Example I

After the initial image has been produced in the emulsion by suitable exposure of a light-sensitive silver bromide gelatin emulsion and the latent image has been developed, but before the image has been fixed, the emulsion is treated with a mild oxidizing agent, such, for example, as a 5-10% solution of cupric chloride, which acts to form the developed silver image into silver chloride. The emulsion is then washed, and the silver chloride is dissolved by a medium which does not dissolve silver bromide. For this purpose a saturated solution of sodium chloride is used, and it has been found that this treatment results in the dissolution of the silver chloride in 5 to 20 minutes, depending upon the strength of the image. After the silver chloride has been dissolved out, the remaining silver bromide is developed in the usual manner to form the reversal silver image.

Instead of using cupric chloride as an oxidizing agent, I might use a 2-5% solution of potassium ferricyanide containing 2-5% of sodium chloride for the purpose of converting the silver image to a silver salt. In this specification the term "mild oxidizing agent" characterizes a solution such as copper chloride or a dilute solution of potassium ferricyanide and sodium chloride. Such solutions are indifferent to the extent that they do not affect the gelatin emulsion, or the support, or destroy dyes or dye-forming substances forming part of a photographic material which is treated in the solutions. In addition, they are indifferent in that they do not affect the sensitivity of the undeveloped silver bromide to as great an extent as the conventional acidic potassium permanganate or bi-chromate solutions previously used as bleaches in the reversal process.

By the use of the above cupric chloride bleach and treatment with a concentrated solution of

sodium chloride, the reversal of the silver image is accomplished in completely neutral or indifferent solutions, thus avoiding the use of strong acid reactions and energetic oxidizing agents.

My invention is not limited to the use of a concentrated sodium chloride solution for the purpose of removing the silver chloride resulting from bleaching the initial silver image. Any other completely neutral solution of a substance can be used which dissolves the silver chloride under complex formation and leaves the unexposed silver bromide undissolved. In the same manner, instead of using a solution of cupric chloride or potassium ferricyanide and sodium chloride for the purpose of converting the silver image into a silver chloride image, any other mild oxidizing agent could be used which operates to convert the silver into a silver salt which is dissolved more readily under complex formation than silver bromide. For example, the developed silver might be transformed into silver rhodanide in the well known manner.

All of these solutions have the common property that they do not affect the gelatin. Likewise, if the emulsion is coated on a paper support, they do not affect the paper fiber. Furthermore, the practice of the process comprised in my invention has the added advantage that the sensitivity of the silver bromide is influenced to a smaller extent than it would be in the case of treatment with bichromate or permanganate. It is, therefore, especially suitable in those photographic processes where the emulsion is again exposed prior to the second development.

My invention is equally applicable to a single layer, or to multilayer materials such as multilayer multicolor photographic material. More particularly, it is applicable to emulsions containing coloring substances distributed uniformly therein which coloring substances are defined for the purposes of this specification and the appended claims as dyes, or dye-forming substances such as those used for color development or for the formation of azo dyes, or leuco esters as described in my U. S. Reissue Patent No. 21,513 and U. S. Patent No. 2,071,688. In the case of layers containing substances for coloring such as dyes or color-forming substances, the full advantages of my improved method are realized in that the silver image can be converted into a reversal image without affecting these dyes or color-forming substances as is disclosed in the following examples:

#### Example II

On a paper support is placed a red sensitized silver bromide emulsion containing 0.3 g. per square meter of Diamine Pure Blue F. F. (Schultz—seventh edition, No. 511) distributed uniformly therein and a green sensitized silver bromide emulsion is placed on top thereof containing 0.4 g. per square meter of Sirius-Rubin B (Ullmann—Enzyklopädie der Technischen Chemie, vol. 9, page 524). An uppermost layer of silver bromide emulsion containing 0.5 g. per square meter of Xylenwalgelb G (Schultz, seventh edition, volume II, page 322) is placed upon the green sensitized emulsion. The dyes are previously precipitated in the emulsions according to the disclosure of co-pending application Serial No. 297,770 of Paul Dreyfus. The layers are exposed through color separation negatives and the silver images developed in each of the layers. The multi-layer material is then treated in a bleaching bath consisting of a 5 to 10% solution of cupric chloride for a period of 5 to 10 minutes

which transforms the silver image in each of the layers into silver chloride. After washing, the material is treated in a saturated solution of sodium chloride for 10 to 20 minutes. During the treatment the silver chloride is dissolved by the formation of a complex. By this treatment the silver images in each of the layers are removed and the remaining silver bromide remains unaffected throughout the treatment. In addition, the dyes present in the layers are not destroyed or otherwise affected by the treatment. After the silver chloride is dissolved, the remaining silver bromide is diffusely exposed or fogged, then developed, and the layers are then subjected to a local dye-destroying treatment, such, for example, as disclosed in my United States Patent No. 2,020,775 dated November 12, 1935. By this treatment a multi-color image is obtained. The remaining silver may be removed by treating the material as previously set forth or it can be removed in accordance with the process described in my United States Patent No. 2,042,253 dated May 26, 1936.

#### Example III

A silver bromide layer containing uniformly distributed therein 1 g. per square meter of the sulfate ester salt of the leuco-compound of (A) hexa-brom-indigo or (B) 6,6'-di-brom-dimethyl-bis-thionaphthene indigo is coated on a reflecting or transparent support. The material is exposed by printing through a negative or by direct exposure in a camera. The material is then treated in accordance with Example I except that after the second development the dye image is formed by the methods disclosed in my United States Reissue Patent No. 21,513 granted July 23, 1940. More particularly, I prefer to transform the silver image into a dye image by the use of a fresh solution consisting of 1/10% potassium bichromate and 1% of hydrobromic acid. After 5 to 10 minutes treatment a reversal blue dye image is formed in the layer if the material contains the compound designated by (A) and a reversal magenta dye image will be formed in the layer if it contains the compound designated by (B). After this treatment the silver and also the unused leuco compound is removed in an alkaline treating bath preferably one containing a small quantity of acetone or methyl alcohol. The reversal treatment preceding the transformation of the silver image to the dye image does not oxidize the leuco compounds to the dye as would result if the known acid bichromate and permanganate silver bleach solutions were employed.

#### Example IV

A material is prepared by coating a film or paper support with a light-sensitive silver bromide emulsion containing uniformly distributed therein 1 g. per square meter of (3,3') dimethyl 1,1' diphenyl 4-4' di-pyrazolone. The material is exposed and then developed in any ordinary developer and afterwards treated with the silver bleach and sodium chloride solution set forth in Example I. The second development is carried on with the following color-forming developing solution:

|                                |     |       |
|--------------------------------|-----|-------|
| Diethyl para-phenylene diamine | g.  | 1     |
| Sodium carbonate (anhydrous)   | g.  | 20    |
| Sodium sulfite                 | g.  | .5    |
| Water                          | cc. | 1,000 |

By this treatment a reversed magenta dye image and a silver image is formed. After washing, the silver image is removed by treating the material

with Farmer's reducer whereby the reversed dye image remains in the layer. The above example is illustrative of a color-developing coupler contained in a photographic layer which is sensitive to powerful oxidizing agents but which is unaffected by the reversal method of this invention. The same treatment could be employed if one or more color developing couplers, each of which is sensitive to conventional oxidizing agents used in known reversal methods, were employed in a multi-layer material.

I have herein shown and particularly described certain embodiments of my invention and certain methods embraced therein for the purpose of explaining its principle and its application, but it will be obvious to those skilled in the art that many modifications and variations are possible. I aim, therefore, to cover all such modifications and variations as fall within the scope of my invention which is defined in the appended claims.

What I claim is:

1. A method of producing a reversal dye image in a light-sensitive silver halide emulsion containing a developed silver image and an easily destroyable coloring substance distributed uniformly therein, which comprises the steps of treating said emulsion with a mild oxidizing agent which converts said developed image to a silver salt image other than the silver halide comprising said light sensitive emulsion without destroying the uniformly distributed coloring substance and subsequently treating the silver salt image with a completely neutral solution comprising a concentrated solution of alkali chloride to dissolve said silver salt image by formation of a complex without affecting the undeveloped silver halide or destroying the coloring substance.

2. A method of producing a reversal dye image in a light-sensitive silver bromide emulsion containing a developed silver image and an easily destroyable coloring substance distributed uniformly therein, which comprises the steps of treating said emulsion with a mild oxidizing agent which converts said developed image to a silver salt image other than silver bromide without destroying the uniformly distributed coloring substance and subsequently treating the silver salt image with a completely neutral solution comprising a saturated solution of sodium chloride to dissolve the silver salt image by formation of a

complex without affecting the undeveloped silver bromide or destroying the coloring substance.

3. A method of producing a reversal dye image in a light-sensitive silver bromide emulsion containing a developed silver image and an easily destroyable coloring substance distributed uniformly therein, which comprises the steps of treating said emulsion with a solution of cupric chloride to produce a silver chloride image without destroying the uniformly distributed coloring substance and subsequently treating the silver chloride image with a completely neutral solution comprising a saturated solution of sodium chloride to dissolve the silver chloride image by formation of a complex without affecting the undeveloped silver bromide or destroying the coloring substance.

4. A method of producing a reversal dye image in a light-sensitive silver bromide emulsion containing a developed silver image and an easily destroyable coloring substance distributed uniformly therein, which comprises the steps of treating said emulsion with a solution of potassium ferricyanide and sodium chloride to bleach said image by forming a silver chloride image without destroying the uniformly distributed coloring substance and subsequently treating the silver chloride image with a completely neutral concentrated solution of alkali chloride to dissolve the silver chloride image by formation of a complex without affecting the undeveloped silver bromide or destroying the coloring substance.

5. A method of producing a reversal dye image in a light-sensitive silver bromide emulsion containing a developed silver image and an easily destroyable coloring substance distributed uniformly therein, which comprises the steps of treating said emulsion with a solution of potassium ferricyanide and sodium chloride to bleach said image by forming a silver chloride image without destroying the uniformly distributed coloring substance and subsequently treating the silver chloride image with a completely neutral salt solution comprising a concentrated solution of sodium chloride to dissolve the silver salt image by formation of a complex without affecting the undeveloped silver bromide or destroying the coloring substance.